

## UNITED STATES PATENT OFFICE

1,929,189

## RAILROAD CAR JOURNAL OIL

Thomas F. Ott, Berkeley, Calif., assignor to  
 Union Oil Company of California, Los Angeles,  
 Calif., a corporation of California

No Drawing. Application December 22, 1931  
 Serial No. 582,645

4 Claims. (CL 87—9)

This invention relates to a lubricating oil which is adaptable for use during extreme temperature conditions. More particularly, it relates to a lubricant such as a railroad car journal oil which is capable of efficient operation at temperatures varying from 100° F. or higher to —50° F. or lower.

An object of this invention is to produce all-weather lubricating oil whose efficiency is unimpaired at the extreme temperature ranges to which lubricants such as railroad car journal oils are sometimes subjected.

Another object is to produce a lubricant whose viscosity does not increase to so great an extent by cooling as to render it unfit for use at low temperatures. Furthermore, its viscosity does not decrease to so great an extent by heating as to harmfully affect its lubricating properties at high temperatures.

20 Another object is to produce a lubricating oil having a very low pour test, for instance, a lubricating oil having a pour point of —60° F. or below and which also has sufficient viscosity at 100° F. to operate efficiently when subjected to 25 temperature of about 100° F. or higher.

Another object is to produce a lubricating oil which has a Saybolt Universal viscosity at 0° F. not above 2000 seconds, a viscosity at 100° F. not below 70 seconds and a pour point not above 30 —60° F.

An additional object is the production of a lubricating oil such as a railroad car journal oil by blending a mineral oil with a fatty oil whereby the inherent lubricating properties of the mineral oil are enhanced by increased oiliness and film stability and by a decreased coefficient of friction.

Up to the present time lubricating oils produced for use at summer temperatures, e. g. 40 100° F. or higher, are relatively inefficient for use at low temperatures because the viscosity rapidly increases with a temperature decrease to the extent that its lubricating value, or "oiliness" becomes negligible. Conversely, up to the present 45 time, the oils destined for use as lubricants at winter temperatures could not be efficiently employed at high temperatures because of the extreme fluidity of these oils at high temperatures. These difficulties are especially apparent when a 50 lubricant must be used under conditions in which large temperature fluctuations occur. For instance, the lubricating oil in railroad car journals must be adaptable for efficient service under wide and varied temperature conditions and must 55 be capable of satisfactorily operating even when

the atmospheric temperature varies quickly and severely.

It is well known that railroad car journals are lubricated by oil absorbed in cotton waste or the like and that the failure of the lubricant results in hot boxes with their consequent delays and dangers. If oil adaptable only for cold weather is employed, an increase in temperature reduces the viscosity of the oil to so great an extent that it becomes too fluid and loses its necessary property of oiliness. If oil adaptable only for warm weather is used, a decrease in temperature increases its viscosity and the cotton waste or other stuffing in the stuffing box balls or rolls and the car journal cannot be properly lubricated. In order to ensure that the oil will lubricate at the low temperatures I have found it advisable to devise an oil which has an extremely low pour point. This will ensure fluidity at these very low temperatures.

Another object of my invention, then, is to produce a railroad car oil which does not have these objectionable characteristics and which operates efficiently at both high and low temperatures.

Another difficulty encountered up to the present time is that lubricating oils change their characteristics during use as lubricants, particularly during use at high temperatures, whereby the lubricating qualities of the oil deteriorate. It is believed that oxidation of the oil is responsible for the gum formation and other changes that occur and for the deleterious reactions which take place within the oil.

A further object, then, is to make a lubricating oil which does not have a tendency to change in characteristics during use, as by oxidation while in service.

An additional object is to economically produce a lubricating oil having these desirable characteristics.

My invention relates to a lubricant which has a relatively flat viscosity curve under extremes of temperature; that is, a lubricant whose viscosity remains relatively unaffected by temperature changes. It has a sufficient body or viscosity at high temperatures, such as 100° F. or higher, to properly lubricate at the temperature and the same oil also has the ability to lubricate as a fluid at low temperatures such as —50° F. at which temperatures the viscosity of the oil has not increased to such a degree as to impair its lubricating value. Previously, cold weather railroad car journal oils at 0° F. had a viscosity as high as 10,000 seconds Saybolt or even in excess of this

figure. My lubricating oil may have a viscosity at 0° F. of 2000 seconds Saybolt or less and a viscosity not below 70 seconds Saybolt at 100° F. In other words, it is not necessary that the viscosity of my lubricating oil be abnormally high at 0° F. in order that it may be of sufficient viscosity at high temperatures such as 100° F. Furthermore, my lubricating oil having these viscosity characteristics may have a pour test not above 10 -60° F. Therefore, it is not necessary that the viscosity of my lubricating oil at 100° F. be abnormally low in order that it may have a pour test below -60° F.

This new and improved lubricant is prepared 15 by blending a mineral oil with a fatty oil. The components of this lubricant have been selected for their special qualifications which give to the final product those characteristics set forth above in the objects of this invention. Preferably, the 20 mineral oil to be blended has a viscosity of 50 to 65 seconds Saybolt Universal at 100° F., for instance 57 seconds at 100° F. and its viscosity at 0° F. is about 1000 seconds Saybolt. The mineral oil remains fluid at -30° F. or lower.

25 The fatty oil which I may employ may be a blown fatty oil such as blown rapeseed oil. As stated above, the presence of fatty oil enhances the inherent lubricating properties of the mineral oil by increasing the oiliness and film stability 30 and by decreasing its coefficient of friction. This fatty oil may have a viscosity of from 1000 to 2000 seconds at 210° F. The use of such fatty oil in blending my lubricant enables me to employ a mineral oil having relatively high viscosities at 35 higher temperatures, such as 100° F. and yet obtain a lubricant having a low pour test. Stated differently, by blending a fatty oil, preferably blown, with a selected mineral oil, I am enabled 40 to produce a lubricating oil having efficient lubricating value at either low or high temperatures.

I have found that lubricants comprising fatty oils mixed with mineral oils are subject to oxidation, especially when used at high temperatures, and that the lubricating value of the composition 45 is thereby greatly diminished because of the formation of gums and oxidation products. In order to prevent these deleterious results, I may employ an oxidized or blown fatty oil in admixture with a mineral lubricating oil. The use of a previously oxidized or blown oil decreases the tendency to further oxidize during use.

Another manner in which I may prevent oxidation of the oil is to employ a mineral oil especially selected for its ability to withstand oxidation at 55 high temperatures. This oil may be compounded with a fatty oil or with an oxidized fatty oil to produce a lubricant having the desired qualities.

Many mineral oils tend to oxidize when exposed 60 to high temperatures for a short time, or even when exposed to moderate temperatures over a long period. In order to maintain the characteristics of the mineral oil during the use of the lubricant at these temperatures, I prefer to select a mineral oil which is not easily oxidized and 65 whose characteristics are not easily changed by use. I have discovered that a suitable mineral oil having these qualifications can be obtained by the well known treatment of mineral lubricating oil with liquid sulphur dioxide as, for instance, 70 in the manner disclosed by Lazar Edeleanu in the United States Patent No. 911,553, issued Feb. 2nd, 1909. This treatment removes substantially all of the unsaturated and aromatic compounds which, I believe, are the components in mineral oil 75 which are the most subject to oxidation or change

during use. I have also discovered that the removal of such compounds from mineral oil also affects the relationship between the viscosity and temperature of the oil, thereby producing an oil that possesses a lesser tendency to thicken or increase in viscosity as the temperature is reduced.

80 In some cases it may not be necessary, in operating according to my invention, to use mineral oil which has been subjected to treatment with liquid sulphur dioxide. This, however, is my preferred embodiment especially when my oil is obtained from naphthenic base crudes such as California asphalt crude. Thus, the petroleum lubricating oil which I blend with fatty oil may be that portion of lubricating oil obtained from naphthenic base crude oils which is substantially insoluble in liquid sulphur dioxide. Untreated mineral oil may be compounded with oxidized or blown fatty oil and good results can be obtained. Also, a mixture of unoxidized and oxidized fatty 90 oil may be employed with mineral lubricating oil which may or may not have been subjected to treatment with liquid sulphur dioxide. Also, a mixture of mineral oil with an unoxidized fatty oil 95 could be used by proper selection of the type and amount of fatty oil employed. Each and all of these modifications are within the purview of my invention.

100 By the term "fatty oils", I mean to include animal, vegetable or fish oils such as cottonseed oil, lard oil and the like. One or more of these oils may be selected for blending with the mineral oil. In my preferred composition, I select oxidized rapeseed oil. The fatty oil may be oxidized in the usual manner, as for instance, by air blow- 110 ing to produce blown oil.

115 As an example illustrating the composition of my lubricating oil, I may blend a mineral oil having a viscosity of 57 seconds at 100° F. and of 1000 seconds at 0° F. and a pour point not above 120 -30° F., for instance -40° F. with 6% of an oxidized or blown rapeseed oil having a viscosity above 1000 seconds Saybolt Universal at 210° F.; for instance, having a viscosity of 1500 seconds Saybolt Universal at 210° F. This mixture exhibits a viscosity of 72 seconds at 100° F. and a viscosity of 1700 seconds at 0° F. This oil also has a pour test of -70° F. The mineral oil may or may not have been treated with liquid sulphur dioxide prior to blending with the oxidized fatty 125 oil. In general, I have found that mineral oil which has been freed from unsaturated and aromatic bodies is superior to oil which has not been subjected to this treatment. It is, of course, evident that the example may be widely varied and 130 yet be within the scope of my invention.

135 In addition, by employing an oxidized fatty oil, such as oxidized rapeseed oil, in admixture with a low viscosity mineral oil obtained from naphthenic base crudes such as California asphalt 140 crudes, I have discovered that it is possible to produce a lubricant whose viscosity is lower at 0° F. and higher at 210° F. than the viscosity of a straight mineral oil having the same viscosity at 100° F. as the viscosity of the blend at 100° F. By a straight mineral oil, I mean one which is unblended with a fatty oil or a blown fatty oil.

145 For instance, a straight mineral oil obtained from California asphaltic crude oil, untreated with sulphur dioxide, may have a viscosity of 3300 seconds at 0° F., 72 seconds at 100° F. and 35 seconds at 210° F. Such an oil may have a pour test not below -55° F. A straight California mineral oil, treated with liquid sulphur dioxide, as described above, for removal of aromatic and un- 150

saturated compounds having the same viscosity of 72 seconds at 100° F. may have a viscosity of 2200 seconds at 0° F. and 36 seconds at 210° F. This oil may have a pour test of -55° F. My 5 blended oil, also having the same viscosity of 72 seconds at 100° F., may have a viscosity of 1700 seconds at 0° F. and 37 seconds at 210° F. This oil may have a pour test of -70° F. or lower. Thus, it is also evident that I can produce a 10 lubricating oil whose pour test is lower than the pour test of a straight mineral oil having the same viscosity at 100° F. as the blend. Furthermore, in addition to the fact that the sulphur dioxide treatment of the California asphalt base mineral 15 oil component of my blend removes the unsaturated and aromatic bodies and thereby produces a mineral oil which is not so readily oxidizable, there is also the added advantage that the sulphur dioxide treatment enables me to use a mineral oil whose viscosity at high temperatures is 20 relatively high and yet which is not excessively viscous at low temperatures and whose pour point is low. When such an oil is blended with fatty or blown fatty oils, the viscosity at high temperatures is maintained or even increased while the 25 viscosity at low temperatures is reduced and the pour point of the blend is lower than the pour point of the mineral oil alone.

The temperature at which an oil congeals is 30 commonly referred to as its pour point and the values recited herein have been obtained according to method D 97-27 T of the American Society of Testing Materials. The measurements of viscosity referred to herein are based upon the 35 American Society of Testing Materials, method D 88-26, using a Saybolt Universal viscosimeter.

It will be understood that the foregoing is

merely illustrative of a preferred operation of the invention, of which many variations may be made by those skilled in the art without departing from the spirit thereof.

I claim:

1. A lubricant comprising a mineral oil and a small quantity of a fatty oil, said mineral oil being substantially insoluble in liquid sulphur dioxide and characterized by a viscosity within the range of approximately 50 to 65 seconds Saybolt Universal at 100° F. and a pour point not above approximately -30° F., and said lubricant being characterized by a maximum Saybolt Universal viscosity at 0° F. of approximately 2000 seconds, a minimum Saybolt Universal viscosity at 100° F. of approximately 70 seconds, and a pour point not above approximately -60° F.

2. A lubricant as defined in claim 1 wherein the fatty oil is an oxidized fatty oil.

3. A lubricant as defined in claim 1 wherein the fatty oil is an oxidized rapeseed oil.

4. A railroad car journal lubricant comprising approximately 6 parts by weight of a blown fatty oil having a viscosity within the range of 1000 to 2000 seconds Saybolt Universal at 210° F. and 94 parts by weight of a mineral oil which is substantially insoluble in liquid sulphur dioxide, which has a viscosity within the range of 50 to 65 seconds Saybolt Universal at 100° F., and which has a pour point of not above -30° F., said lubricant being characterized by a maximum Saybolt Universal viscosity at 0° F. of approximately 2000 seconds, and a minimum Saybolt viscosity at 100° F. of approximately 70 seconds, and a pour point not above approximately -60° F.

THOMAS F. OTT.

40

115

45

120

50

125

55

130

60

135

65

140

70

145

75

150

80

85

90

95

100

105

110

120

125

130

135

140

145

150